

# UNITED STATES PATENT OFFICE.

PASCAL MARINO, OF LONDON, ENGLAND.

PROCESS OF PREPARING ELECTROLYTES FOR USE IN THE DEPOSITION OF A METAL OR METALLIC ALLOY.

1,073,432.

Specification of Letters Patent. Patented Sept. 16, 1913.

No Drawing.

Application filed October 29, 1912. Serial No. 728,400.

To all whom it may concern:

Be it known that I, PASCAL MARINO, a subject of the King of Italy, and resident of 129 Albert street, Park street, London, N. W., England, professor of chemistry, have invented a certain new and useful Process of Preparing Electrolytes for Use in the Deposition of a Metal or Metallic Alloy, of which the following is a specification.

10. The object of the present invention is to facilitate the electro-chemical reduction of soluble metal salts into ions by dissociating said salts as completely as possible in order to subsequently electrolytically deposit 15 the metal present in said salts on metallic or metallized surfaces, and to produce alloys such as those of nickel and silver or of tin and copper (bronze) by the simultaneous electrolytic deposition of the metals 20 constituting those alloys. I refer more particularly to these alloys as they are of considerable commercial importance owing to their extensive use in the arts, their durability, and the resistance they offer to atmospheric influences. This disassociation is effected by submitting the solution of the salts to the herein described process which is constituted by three following successive steps, viz:—(a) I add to a solution of the 25 salt or salts of the metal or metals to be deposited, an organic reducing agent which serves to effect the partial dissociation of the metallic salt or salts. (b) I then heat the solution in order to assist in the dissociation by decreasing the cohesion of the molecules and thus overcoming certain affinities irreducible at ordinary temperatures. (c) When the solution has become cold I add to it another reducing agent for the purpose of 30 effecting dissociation to a maximum degree, that is, as far as may be without altering the fact of solution.

Owing to the dissociation of the soluble metal salts these salts are resolved into ions 45 which serve as current carriers. When the dissociation has been effected the molecular conductivity of the electrolyte is at its maximum, and hence it is easy to effect the reduction of the solution forming the electrolyte 50 by a relatively weak current, (as only solutions containing ions are conductors of electricity,) and to obtain a pure, metallic,

homogeneous, electrolytic deposit which tenaciously adheres to the cathode.

As regards the organic reducing agents 55 it is necessary to employ an organic acid combined with a fixed base in order to assure the stability of the electrolyte. As reducing agent during the first step of the process I prefer to employ magnesium borocitrate in solution. As regards the reducing agent during the last step of the process I prefer to employ either gluco-citric or gluco-tartaric acid in the proportion of 15% of the weight of the metal salt or salts. 60 Gluco-citric acid may be prepared by mixing together 1 molecular weight of glucose and 3 molecular weights of citric acid, and gluco-tartaric acid by mixing together 1 molecular weight of glucose and 2 molecular 65 weights of tartaric acid.

In carrying out my invention, it is necessary to select a salt of the metal to be deposited which will become wholly dissolved in the electrolyte and yield a pure metallic 70 deposit.

It is to be understood that my invention is not limited to the deposition of any particular metal or metallic alloys and I will now refer to certain metals by way of example and to the salts of these metals which I prefer to use, premising that in making a selection of the salts care must be taken to avoid mixing with the magnesium borocitrate solution, metallic solutions which 80 would, when in presence, decompose one another and form an insoluble compound.

Inasmuch as potassium cyanid is a solvent for gold, silver, nickel, and copper, there should be employed when these metals 90 or their alloys are to be deposited either gold, silver, nickel or copper cyanid of potassium salts. For depositing iridium I prefer to use iridium chlorid, as a solution of this salt yields by electrolysis a pure metallic deposit. For depositing palladium, it is necessary to employ palladium-chlorid which I dissolve in ammonia to form palladium-ammonium-chlorid. For depositing rhodium, I prefer to employ rhodium-sodium-chlorid. For depositing platinum, it is preferable to use a solution of potassium 100 platinate. This solution should be so perfectly neutral that, when diluted in dis-

tilled water, it will not alter the color of litmus paper which has been previously reddened by immersion in an acid.

Tin is a metal difficult to reduce owing to the fact that its transition from its spongy to its crystalline state is so rapid that it is almost impossible to obtain a notable deposit of the metal in a ductile and malleable state. For depositing tin I prefer to employ tin sulfate dissolved in aluminium sulfate neutralized by barium chlorid. For depositing iron I prefer to employ iron protochlorid which is a neutral salt. For depositing cadmium or zinc I prefer to employ ammonium-sulfate salts of said metals in order to obtain a malleable and ductile deposit. A solution of the salts of these metals possesses high conductivity and zinc or cadmium anodes dissolve in it very easily. For depositing lead I prefer to employ a lead salt dissolved in ammonium tartrate in order to obtain a homogeneous metallic deposit. For depositing tungsten, it is necessary first to prepare a solution of an alkaline tungstate and then to pour it drop by drop into diluted nitric acid. The tungsten compound thus obtained is then dissolved in ammonium tartrate mixed with potassium or sodium phosphate. For depositing chromium, there must be employed chromium sulfate dissolved either in potassium or aluminium sulfate. For depositing molybdenum I prefer to employ ammonium phosphomolybdate dissolved in potassium hydroxid.

35 The organic reducing agent first employed should in all cases be capable of remaining unaffected by heat.

In order to obtain the simultaneous electrolytic deposit of an alloy, the electrolyte 40 may be prepared by treating a mixture of the metals according to the method above set forth, or by treating each metal separately to obtain separate electrolytes and afterward mixing the electrolytes together. 45 In this connection I would state that consideration must be given to the relative proportions of the individual metals necessary to obtain the desired alloy, to the law of precipitation of each individual metal, and 50 to the amount and density of current necessary for satisfactorily depositing a stated quantity of metal per ampere-hour which depend on the electro-chemical equivalency of each metal. As the electrolytes for depositing alloys are similarly prepared, a mixture of them will be of a stable nature 55 and will not form an insoluble product.

It is obviously unnecessary to give directions regarding the actual deposition process 60 as this in no way varies from current practice.

When in the appended claims I speak of gluco-citric acid, I desire to include also its well-known equivalents, such as gluco-tar-

taric acid. It will be further understood 65 that when I speak of the metal to be deposited, I mean to include a mixture of metals, as in the form of an alloy, and when I refer to a salt of the metal, I mean to include salts of the metals forming the mixture. 70

Having now particularly described and ascertained the nature of the said invention and in what manner the same is to be performed, I declare that what I claim is:— 75

1. The process of preparing an electrolyte for use in the deposition of a metal, which consists in first making a suitable aqueous solution containing a salt of the metal to be deposited, then adding a suitable organic reducing agent to the solution, then heating the resulting liquid, and finally, when said liquid has cooled, adding to it a suitable organic reducing agent, substantially as and for the purpose described. 85

2. The process of preparing an electrolyte for use in the deposition of a metal, which consists in first making a suitable aqueous solution containing a salt of the metal to be deposited, then adding magnesium-boro-citrate to said solution, then heating the resulting liquid, and finally, when said liquid has cooled, adding to it a suitable organic reducing agent, substantially as and for the purpose described. 90

3. The process of preparing an electrolyte for use in the deposition of a metal, which consists in first making a suitable aqueous solution containing a salt of the metal to be deposited, then adding a suitable organic reducing agent to the solution, then heating the resulting liquid, and finally, when said liquid has cooled, adding to it a suitable quantity of gluco-citric acid, substantially as and for the purpose described. 100

4. The process of preparing an electrolyte for use in the deposition of a metal, which consists in first making a suitable aqueous solution containing a salt of the metal to be deposited, then adding magnesium boro-citrate to said solution, then heating the resulting liquid, and finally, when said liquid has cooled, adding to it a suitable quantity of gluco-citric acid, substantially as and for the purpose described. 110

5. An electrolyte for use in the deposition of a metal, comprising a solution containing a salt of the metal to be deposited, said salt being dissociated to a maximum degree into ions by the treatment of a suitable aqueous solution containing said salt with a suitable organic reducing agent, then heating the resulting liquid, and finally, when said liquid has cooled, adding to it a suitable organic reducing agent, substantially as and for the purpose described. 120

6. An electrolyte for use in the deposition of a metal, comprising a solution containing

a salt of the metal to be deposited, said salt being dissociated to a maximum degree into ions by the treatment of a suitable aqueous solution containing said salt with magnesium boro-citrate, then heating the resulting liquid, and finally, when said liquid has cooled, adding to it a suitable quantity of gluco-citric acid, substantially as and for the purpose described.

PASCAL MARINO.

Witnesses:

WILLIAM DAVIES,  
O. J. WORTH.